

March 17, 1942.

G. LAUBMEYER

2,276,583

ELECTRIC HEATING ELEMENT

Filed June 23, 1939

Fig. 1.



Fig. 2.



Fig. 3.



Fig. 4.



Fig. 5.



Inventor:

Günther Laubmeyer,

Bailey & Larson  
Attorneys

## UNITED STATES PATENT OFFICE

2,276,583

## ELECTRIC HEATING ELEMENT

Günther Laubmeyer, Kassel-Wilhelmshohe,  
GermanyApplication June 23, 1939, Serial No. 280,885  
In Germany June 30, 1938

5 Claims. (Cl. 201—67)

This invention is directed to an electrical resistance heating element. More particularly, the invention is directed to the construction of the electrical heating element of a material not readily oxidized.

Electrical resistance heating elements adapted to operate under heavy load at high temperatures have generally heretofore been constructed upon a core of substantially pure nickel, or nickel-steel alloys, or other expensive steels, such as V2A nickel-chromium steel. Because of the high temperatures developed in the heating elements, ordinary inexpensive metals such as iron oxidize to such an extent that the layers of oxidized material developed upon the core eventually build up to the point where the electrical conductors break under pressure and consequently the heating element fails.

The art has long searched for a substitute for the expensive pure nickel used to form the cores of the resistance elements. Nickel-steel alloys are not satisfactory as they are likewise expensive and are, moreover, difficult to work into desired shapes. Heretofore, a satisfactory core made of cheap, easily worked material has not been discovered.

It is an object of this invention to construct a heating element having a core made of low cost metals, which core is resistant to oxidation under high temperatures.

Another object of the invention is to find a satisfactory substitute for the expensive pure nickel and alloy nickel-steel cores used for making high temperature electrical resistance heating units.

Another object of the invention is to produce a resistance heating element having either a circularly wound or a flatly wound resistance coil supported upon a core of cheap material not greatly oxidized at high temperatures.

Generally these objects are obtained by constructing an iron core having an aluminum alloy surface produced by diffusion welding.

Both aluminum and iron are relatively cheap materials, especially when compared with expensive chrome or nickel-steel alloys, and both the iron and aluminum are, by themselves, ordinarily unusable for the formation of high temperature heating elements. Iron by itself oxidizes excessively at high temperatures, and aluminum by itself is too soft. However, an aluminum iron alloy has strength and low oxidation characteristics at high temperatures and consequently produce a satisfactory material. The alloy can be obtained by forming layers

of aluminum around the iron core, and then producing a diffusion welding between the aluminum and the surface of the iron core by completing the resistance element and bringing it to a temperature at which the diffusion between the iron and aluminum takes place, or by inserting the core covered with aluminum into a mold and heating this mold to the diffusion temperature. Care is exercised to make sure that the aluminum reacts with the iron alone.

10 The means by which the objects of the invention are obtained may be more fully understood with reference to the accompanying drawing, in which:

15 Fig. 1 is a cross view of a heating element constructed according to this invention.

Fig. 2 is a cross sectional view of the core having the layers of aluminum applied thereto.

20 Fig. 3 is a cross sectional view on the line 3—3 of Fig. 2.

Fig. 4 is a view corresponding to Fig. 3, but showing the aluminum layer after diffusion has taken place between the aluminum and the iron.

25 Fig. 5 is a cross sectional view of the core with the aluminum layers such as shown in Fig. 3 inserted within a mold.

30 In Fig. 1 the iron core 10 is coated with an aluminum layer 12. The iron core is shown as a tube of circular section with outwardly flared ends. Obviously tube 10 may be of oval, or polygonal, section, and may be solid. The surface of the core 10 is cleaned of oxide by ordinary methods, such as brushing, grinding, or scouring.

35 The aluminum layer 12 can be applied in the form of thin flexible sheets, or layers of foil. A plurality of layers are usually applied, inasmuch as under long, continual heating, the aluminum eventually becomes entirely diffused throughout

40 the iron, and the greater the quantity of aluminum initially applied means that the life of the unit will be longer. The aluminum layers are tightly wound about the core 10.

45 The electrical conductors 16 are wound about the aluminum coated core, these wires being separated by mica insulation 18. The electrical leads to the coils 16 are shown at 20 and 22. A longitudinally split sheet metal sleeve 24 covers the coils 16. This sleeve is wrapped by a steel wire 26. Coil 16 and the externally wrapped wire 26 both aid in pressing the aluminum layer 12 very tightly against the surface of core 10.

50 The heating element thus constructed is then heated through the medium of the resistance of

the coil 16 to an electric current up to or slightly more than the melting point of the aluminum, and at this temperature diffusion takes place between the aluminum and the iron, this diffusion being aided by the externally applied pressure upon the aluminum against the surface of the core, as well as by the expansion of core 10 during the heating. An aluminum iron alloy 14 is thus formed on the exterior of the core, the alloy having a high aluminum content on the outside which gradually decreases toward the interior of the core 10. As aluminum iron alloys are highly refractory, the surface of the core is protected against oxidation at high temperatures, and consequently the heating element is ensured of a long life. A satisfactory substitute for the expensive nickel steels is thus achieved.

In Fig. 5, a second method is shown of producing the core with an aluminum iron alloy surface. The core, with the layers of aluminum thereon as seen in Fig. 3, is inserted between the two halves 28 and 30 of a mold. The halves of the mold are tightened upon the aluminum covered core by means of bolts 32 and nuts 34 and 36, the aluminum coating thus being pressed very tightly against the surface of the core. The mold is then placed in a furnace and the temperature of the core and aluminum raised to the point where the aluminum diffuses with the iron of the core to become alloyed therewith. An insulating layer 38 of mica is inserted between the aluminum 12 and the halves of the core so that no diffusion takes place between the aluminum and the mold.

Instead of a mold such as shown in Fig. 5, a metal sleeve or band could be employed, said sleeve or band being insulated from the aluminum by means of mica or asbestos. The metal band may be wound about the aluminum coated core and after being so wound, tightened so as to press the aluminum tightly against the core. After the core has thus been prepared as shown in Fig. 5, the heating elements 16, as shown in Fig. 1, are applied to the aluminum surface core in order to complete the heating unit.

As has been stated, the core can assume any cross sectional form, and can be either hollow or solid. Likewise, the electrical conductors may be either cylindrically coiled as shown, or may be flatly formed. In any case, an aluminum iron alloy is formed upon the surface of the core so that layers of oxidized iron will not occur during the use of the heating element under heavy loads and high temperatures.

It thus appears that a satisfactory substitute for the relatively expensive nickel and nickel-steel has been obtained. Use has been made of two relatively cheap materials by causing them to be alloyed, and the alloying of the metal can take place as one of the steps in the normal assembly of the elements of the heating unit.

Having now described a means by which the objects of this invention may be obtained, what I claim as new and desire to secure by Letters Patent is:

1. An electrical heating resistance unit comprising an iron core, at least one layer composed of aluminum in sheet form placed on said core, and electrical heating elements firmly contacting said layer to hold said layer to said core whereby an iron-aluminum alloy zone is formed between said core and said layer when said unit is heated during use.

2. An electrical heating resistance unit comprising an iron core, a sheet of aluminum enclosing said core, and insulated electrical heating coils tightly wound upon said sheet to fasten it to said core whereby an iron-aluminum alloy zone is formed between said core and said sheet when said unit is heated during use.

3. An electrical heating resistance unit comprising an iron core, at least one layer composed of an aluminum sheet upon the surface of said core, insulated electrical heating elements contacting said layer, a sleeve enclosing said elements, and means for tightening said sleeve upon said elements to hold said layer in firm contact with said core whereby an iron-aluminum alloy zone is formed between said core and said layer when said unit is heated during use.

4. An electrical heating resistance unit comprising an iron core, at least one layer of aluminum foil upon the surface of said core, and a heating element tightly securing said aluminum layer to said core whereby heating of said unit produces by diffusion an iron-aluminum surface upon said core.

5. An electrical heating resistance unit comprising an iron core, a plurality of layers of sheet aluminum upon said core, insulated electrical heating elements upon said layers, and means for securing and tightly pressing said elements and layers tightly against said core whereby an iron-aluminum alloy zone is formed between said core and said layer when said unit is heated during use.

GÜNTHER LAUBMEYER.